

## UNITED STATES PATENT OFFICE

1,983,918

MANUFACTURE OF WATER-REPELLENT  
PAPERS OR PAPER ARTICLES SIZED  
WITH WAX DISPERSIONSOscar F. Neitzke, Belmont, Mass., assignor to  
Bennett, Incorporated, Cambridge, Mass., a  
Corporation of MassachusettsNo Drawing. Application August 6, 1932,  
Serial No. 627,811

5 Claims. (Cl. 92—68)

Within recent years, great strides have been made in manufacturing water-repellent papers through the addition of aqueous wax dispersions to the paper pulp before it is delivered to suitable paper-forming or board-forming machines. Sized papers or boards thus made are put to various uses, including manufacture into such articles as drinking cups and cartons for vending wet food products, such as oysters, ice cream, or the like.

When the bulk pulp is sized with aqueous wax dispersions, such as paraffin wax, the dispersed particles are fixed on the pulp fibers in the form of discrete, small particles. These particles undergo more or less fluxing and coalescence when the sheet of paper or board formed from the pulp passes over the dry end of the papermaking machine. It must, however, be borne in mind that papermaking machines are run at such high rates of speed that the paper sheet is exposed to elevated temperature for only a matter of seconds. Again, the paper rarely reaches the temperature of the hot drier drums, because during most of its travel over the dry end of the paper machine it is associated with considerable water, which must be evaporated from the sheet before it acquires the temperature of the drums. It is thus seen that when papers are sized through the use of aqueous wax dispersions, as hereinbefore described, their wax content has comparatively little opportunity to become thoroughly fluxed and coalesced as a continuous phase or body in the sheet.

I have found that the degree to which a paper or board containing dispersed wax size acquires water-repellency depends in large measure upon the fluxing and coalescence which its wax content has undergone. Indeed, I have discovered that papers or boards sized as heretofore through the use of aqueous wax dispersions never develop their potential water-resistance on account of the inadequate fluxing action which they have undergone on the papermaking machine. It is hence not surprising that papers or boards so made are highly ineffective against the action of hot, aqueous liquids. For instance, drinking cups made of paper which has been wax-sized by adding aqueous dispersions of wax to the furnish in the beater engine leak almost at once when hot water is poured thereinto. The same is true of cartons made from paperboard which has been sized in a similar way. In other words, although such papers or boards may for some purposes be sufficiently resistant to the penetrating and disintegrating action of cold water, they

are entirely unsatisfactory when subjected to the action of hot water or other aqueous liquids which tend to penetrate and loosen the fibrous structure.

In working to overcome the deficiencies of papers or boards sized with wax dispersions, I have found that it is possible to develop surprisingly high water-repellency therein, provided that the papers or boards, after they have come off the papermaking machine are subjected to a temperature distinctly above the melting point of the wax but short of the scorching temperature of the paper for a substantial period of time, that is, for at least a few minutes. When the paper or board is to be converted into such ultimate articles as drinking cups or cartons, these articles may be subjected to the heat treatment. On the other hand, the paper or board itself may be heat-treated as in the form of rolls or separate sheets. While it is possible to accomplish the desired transformation of the paper or board in a dry atmosphere, it is preferable that the atmosphere be laden with moisture so as to avoid charring and embrittlement of the fibers.

In those cases when the water-repellent paper or board is to serve for the fabrication of such articles as drinking cups or cartons for vending wet edibles, it is common practice to use paraffine wax as the water-repellent material, because it is tasteless and odorless and imparts a softness and pliability to the paper, comporting well with formation into curved or sharp-cornered containers. I shall therefore illustrate the principles of my invention by citing specifically the treatment of a paperboard containing dispersed hydrocarbon wax of the paraffin series as the sizing agent and known in the trade as "can body stock." The board may comprise any suitable fibrous base and contain sizing agents, such as rosin, in addition to the dispersed paraffin wax. Thus, it may contain about 1% to 2% of dispersed hydrocarbon wax and about 3% rosin size as its sizing components. Such board should be exposed for at least about fifteen minutes to a temperature of about 225° to 275° F. in order to acquire a water-repellency consonant with an ability to withstand the disintegrating action of hot, aqueous liquids, e. g., hot coffee or the like. A cup or carton fabricated from board heat-treated in this way can withstand the action of boiling water indefinitely, whereas the same container lacking the heat-treatment is attacked by boiling water and begins to leak at once. Repeated experiments consistently show that cartons or cups made from the heat-treated papers of the present invention are well

adapted to receive boiling coffee or similar aqueous liquids and to hold such liquids until they have cooled to room temperature without any leakage whatever.

- 5 As already indicated, the heating chamber for the paper or board, or the finished articles made therefrom, is preferably kept highly humid, so as to maintain the paper in soft, pliant condition and thereby to avoid an "over-dried" condition associated with irreparable injury to the paper. To this end, it is possible to supply live steam at the proper temperature as the heating medium for the chamber. When hot air is used as the heating medium, it is also preferably commingled with steam vapor, as by emitting steam into the chamber or by maintaining therein shallow trays of water presenting a large evaporating surface. When rolls of paper or board are subjected to the heat treatment, it is important that the rolls reach the desired high temperature uniformly throughout. Depending upon the size of the roll, this may take some hours, but a long period of exposure is beneficial, rather than otherwise. On the other hand, even when the paper is heated in the form of finished articles and thus quickly acquires the desired temperature uniformly throughout, the heating period should be at least about fifteen minutes, since a shorter heat treatment does not develop the maximum potential water repellency therein. In fact, I find it better to expose the finished articles for about one-half hour to an atmosphere heated to a temperature of about 225° to 275° F., in order to ensure what may be termed an equilibrium water-repellency in the paper. In the case of rolls of paper or board requiring an unduly extended heating period to reach a uniform temperature throughout, provision may be made to shorten this period, as by winding the paper on perforated mandrels or cores, through which steam and/or heated air may be circulated so as to effect a heating of the rolls from their interiors, as well as from their outer surfaces.
- 45 It is to be understood that the principles of my invention apply, no matter what kind of paper stock is used in the body of the paper or board. Thus, the stock may advantageously be a mixed furnish containing non-cellulosic fibers, such as asbestos, as well as cellulosic fibers, such as wood pulp, since the papers made from such stock, especially an asbestos-containing paper is vastly improved in its water-repellency when made according to the present invention. Any of the conventional ways of sizing the stock with aqueous dispersions of wax may be adopted. In the case of wax dispersions which contain rosin soap or other precipitable stabilizer, the stabilizer may be reacted upon with alum or other suitable precipitant, so as to cause the deposition of the dispersed wax on the stock before the papermaking step. Any other method of introducing the dispersed wax and other sizing material into the paper may be used. In some instances, the wax dispersion may be applied as a surface size to a prefabricated sheet of paper, as by a spraying, dipping, or coating operation, followed, if desired, by calendering under heavy pressure to force the wax particles into the body of the paper. In such instances, too, I have found that the heat treatment hereinbefore described is of great value, as it develops in the paper its maximum water-repellency impossible of attainment when the surface-sized paper is quickly run through a succession

of calender rolls even in hot condition. I have adverted to the fact that the heat treatment of the present invention as applied to papers sized with dispersed hydrocarbon wax is preferably conducted within a temperature range of about 225° to 275° F. This is especially true in the case of a dispersed hydrocarbon wax having a melting point of about 150° to 160° F. Both the lower and upper temperature limits are of significance in such case, for, if paper sized with such dispersed wax is exposed to temperatures materially below 225° F., it is improved but little in water-repellency even after prolonged exposure, whereas, if the paper undergoes much heating at temperatures considerably in excess of 275° F., it is likely to be badly scorched or discolored and to lose its best physical characteristics.

Paper sized with dispersed wax, other than that specifically mentioned, may be associated with other temperature and time factors, but in each case it is necessary to heat the paper for at least a few minutes distinctly above the melting point of the wax, in order to develop highest water-repellency therein. When water-dispersed waxes whose melting point is lower than 150° to 160° F. are employed for sizing papers or boards as hereinbefore described, one may heat the dried papers or boards to a minimum temperature below 225° F. and yet realize the desired improvement in water-repellency so long as the melting point of such waxes is distinctly overstepped and maintained for a matter of minutes. Thus, when so-called scale wax having a melting point of about 120° F. constitutes the water-dispersed size which is incorporated into papers or boards, one need heat the dried papers or boards to a minimum temperature of only about 160° F. for about fifteen minutes to realize the desired improvement in water-repellency. Of course, one may heat such papers or boards to temperatures above 160° F. to shorten the time period necessary for the attainment of the desired result, so long as one does not exceed a temperature of about 275° F., which, as already indicated, detracts from the best physical characteristics of the papers or boards. With a wax of given melting point, it is preferable to perform the heat treatment on the sized papers or boards at the maximum temperature consistent with a preservation of the physical characteristics of the papers or boards, since the greater the differential between the temperature of the heat treatment and the melting point of the wax, the shorter is the time of heat treatment necessary for the attainment of a given increase in water-repellency in the papers or boards.

There are provinces of utility for my invention other than in producing fabricated articles such as cups and cartons, designed for use in connection with aqueous liquids or wet food products at normal or elevated temperature conditions. There are instances when it is desired that the papers or boards as such acquire the maximum water-repellency attainable through the use of a given amount of water-dispersed wax as a sizing ingredient therein, since such papers may be used for wrapping wet food products, such as vegetables or meats, or may serve in making bags, boxes, or other containers designed to protect their contents against moisture, as well as to resist disintegration in the presence of moisture. For these various uses, papers or boards treated in accordance with my invention are far more satisfactory than similar papers which are used substantially in the condition that they leave the

dry end of the papermaking machine. In the case of wall boards, insulating boards, and similar materials of construction containing dispersed wax and consisting of one or more plies made on a papermaking machine, it is, of course, highly desirable that such boards be made as water-repellent as possible through the use of a given amount of water-dispersed wax, as this means that such boards will be characterized by such 10 importantly desirable qualities as low expansibility and low shrinkability. Such boards may, therefore, advantageously receive the heat treatment of the present invention, in order that their 15 tendency to shrink and warp on account of repeated moistening and drying may be greatly diminished. In the case of plied or built-up boards made by adhesively securing a number of dried plies in superposed face to face relationship, it is possible to subject either the individual plies 20 or the built-up board to the heat treatment of the present invention.

In carrying out investigations to ascertain the effect of a heat treatment such as I have described on papers or boards sized with materials other than wax, and more especially with various 25 rosin sizes lacking wax as a sizing component, it was found that the papers or boards were improved little, if any, in their water-repellency. Apparently such water-repelling effect as can be 30 secured in rosin-sized paper is had when the paper is subjected to drying as ordinarily, that is, as it traverses the dry end of the papermaking machine. When dried, rosin-sized paper is then heat-treated as hereinbefore described, one 35 does not significantly appreciate the water-repellency of the paper, even though the paper may be heated for a considerable period of time at temperatures as high as 225° F. This result is evidently attributable to the fact that the aluminum or other metal resinate invariably occurring 40 in rosin-sized papers along with free rosin renders the size as a whole so refractory or resistant to softening and fusion by the action of heat that it is impossible to enhance the water-repellency of 45 such papers without going to such high temperatures as would discolor and otherwise injure them. What I have said holds true even of papers where-into have entered rosin sizing compositions containing a substantial proportion of free or unsaponified rosin, for instance compositions containing 50 as much as 25% or more free rosin.

In the appended claims, I use the word "paper" in its broad sense to comprehend not only the papers but also thick sheets or boards of one or 55 more plies made on papermaking machinery.

I claim:

1. In the production of papers of high water-repellency containing but a small percentage of sizing material, including wax, those steps which 60 comprise incorporating into paper-making stock an amount of water-dispersed, solid wax and a stabilizer for said dispersed wax to constitute such wax and stabilizer but a small percentage of said stock, running the resulting stock off on a paper-making machine equipped with a dry end and running at a speed such that the resulting paper 65 is delivered in dry condition from the dry end at much lower than its maximum water-repellency, and subjecting the paper in the condition 70 that it leaves the dry end for at least a few minutes to a temperature distinctly above the melting point of the wax but below the scorching temperature of the paper, thereby causing the wax content to become thoroughly fluxed and coa-

lesced on the fibers and enhancing markedly the water-repellency of the paper.

2. In the production of papers of high water-repellency containing but a small percentage of sizing material, including wax, those steps which 5 comprise incorporating into paper-making stock water-dispersed wax and rosin-size-stabilizer for said dispersed wax to constitute such wax and stabilizer but a small percentage of said stock, adding a precipitant to fix the wax and rosin size 10 to the stock, running the resulting stock off on a paper-making machine equipped with a dry end and running at a speed such that the resulting paper is delivered in dry condition from the dry end at much lower than its maximum water-repellency, and subjecting the paper in the condition 15 that it leaves the dry end for at least a few minutes to a temperature distinctly above the melting point of the wax but below the scorching temperature of the paper, thereby causing the 20 wax content to become thoroughly fluxed and coalesced on the fibers and enhancing markedly the water-repellency of the paper.

3. In the production of papers of high water-repellency containing but a small percentage of 25 sizing material, including hydrocarbon wax, those steps which comprise incorporating into paper-making stock an amount of water-dispersing, solid, hydrocarbon wax and a stabilizer for said dispersed wax to constitute such wax and stabilizer but a small percentage of said stock, running the resulting stock off on a paper-making machine equipped with a dry end and running at a speed 30 such that the resulting paper is delivered in dry condition from the dry end at much lower than its maximum water-repellency, and subjecting the paper in the condition that it leaves the dry end for at least about fifteen minutes to a temperature 35 distinctly above the melting point of such wax but below about 275° F., thereby causing the 40 wax content to become thoroughly fluxed and coalesced on the fibers and enhancing markedly the water-repellency of the paper.

4. In the production of papers of high water-repellency containing but a small percentage of 45 sizing material, including hydrocarbon wax, those steps which comprise incorporating into paper-making stock an amount of water-dispersed, solid, hydrocarbon wax and a precipitable stabilizer for said dispersed wax to constitute such wax and 50 stabilizer but a small percentage of said stock, adding a precipitant to precipitate said stabilizer and fix said wax to the stock, running the resulting stock off on a paper-making machine equipped with a dry end and running at a speed 55 such that the resulting paper is delivered in dry condition from the dry end at much lower than its maximum water-repellency, and exposing the paper in the condition that it leaves the dry end for at least about fifteen minutes to a moist atmosphere at a temperature distinctly above the 60 melting point of such wax but below about 275° F., thereby causing the wax content to become thoroughly fluxed and coalesced on the fibers and enhancing markedly the water-repellency of 65 the paper.

5. A water-repellent paper product comprising 70 felted fibers and a small proportion of wax-containing sizing material substantially uniformly distributed by fusion and coalescence over the said fibers, the said product being substantially that resulting from the steps set forth in claim 1.